

1

2,840,891

## HIGH TEMPERATURE STRUCTURAL MATERIAL AND METHOD OF PRODUCING SAME

John S. Nachtman, Washington, D. C.

No Drawing. Application January 4, 1955  
Serial No. 479,874

8 Claims. (Cl. 29—182.5)

(Granted under Title 35, U. S. Code (1952), sec. 266)

The invention described herein may be manufactured and used by or for the Government of the United States of America for governmental purposes without the payment of any royalties thereon or therefor.

This invention relates to structural materials having unusual strength and hardness at elevated temperatures, and methods for the production of such materials.

More particularly, the present invention is concerned with a metallurgical composition comprising inorganic substances, metallic or non-metallic, and a base metal, such as aluminum and alloys of aluminum, and a method of producing structural materials therefrom by utilization of certain techniques of powder metallurgy.

In the prior art, metal oxides, inorganic compounds of mixed metal oxides, and other inorganic non-metallics are usually considered to be detrimental to the useful properties of base metals or metal alloys containing such substances in substantial percentage. This, however, is not always true, and contrary to prior teachings it has been found that the proper amount and distribution of these substances lead to enhanced properties in metals and alloys.

For example, structural materials possessing unusual and desirable properties may be produced by powder metallurgical processes from compositions of aluminum or aluminum alloy powder containing finely divided inorganic additives of substances other than aluminum oxide alone, such as metal oxides, compounds of mixed metal oxides, and other inorganics, both metallic and non-metallic. The structural material produced therefrom and in accordance with this invention are characterized by relatively light weight and greatly improved strength and hardness at elevated temperatures up to about 1200° F.

It is a principal object of this invention to produce compact substantially non-porous aluminum base structural material possessing light weight and greatly improved hardness and strength at temperatures up to about 1200° F.

It is another object of the invention to produce compact substantially non-porous light weight structural materials characterized by unusual strength and hardness at elevated temperatures from compositions comprising aluminum or aluminum alloy powder and finely divided

2

inorganic additives of substances other than aluminum oxide alone.

It is a further object of the invention to provide methods of producing such compact substantially non-porous structural materials from the before mentioned powder compositions by utilization of suitable powder metallurgical techniques.

Still further objects of the invention include compact substantially non-porous structural materials, and forms 10 therefrom, resulting from such powder compositions and methods.

Still further objects and the attendant advantages of the invention will be obvious to those skilled in the art from the more detailed description set forth below, it being understood that the following detailed description is given by way of illustration and explanation only, and not by way of limitation, since various changes therein may be made by those skilled in the art without departing from the spirit and scope of the invention.

20 Broadly stated, the foregoing objects may be accomplished by means of a process comprising the following steps: (1) producing a powder composition comprising aluminum or aluminum alloy powder and a suitable finely divided inorganic additive; (2) milling said powder 25 composition preferably with sufficient wetting agent to form a soft paste; (3) preferably presintering the milled powder composition at about 800° F. under an inert atmosphere, and then cooling to room temperature before exposing to air; (4) utilizing techniques of powder metallurgy to produce a desired form from the before mentioned powder composition.

The process, as briefly set forth above, is hereinafter described with particular reference to producing compacts 35 from a powder composition consisting of approximately 50–95 parts aluminum powder and approximately 5–50 parts titanium dioxide. However, it will be appreciated that the invention is not limited to such compositions or the production of such compacts, and that other well 40 known powder metallurgical techniques may be used to form larger or more complicated shapes from the powder composition resulting from steps (1) through (3).

Regardless of the final form, the structural material produced in accordance with the invention is characterized by light weight, compact relatively non-porous forms of unusually high strength and hardness at elevated temperatures up to about 1200° F. as distinguished from conventional porous ceramics which have low physical strength.

50 Table I gave hardness data for various stages in the processing of compacts and hot hardness data at different testing temperatures. Examples are given therein of compacts composed of aluminum powder, aluminum powder and a metal oxide, aluminum powder and a compound of mixed metal oxides, aluminum powder and a metal, aluminum powder and either a metal sulfide, carbide, boride, or oxygen bearing compounds and mixtures 55 of two or more of the foregoing substances.

TABLE I.—HOT HARDNESS OF ALUMINUM BASE POWDER PRODUCTS

| Percent Additive to Aluminum Powder  |       | Rockwell superficial hardness number, $R_w$ (1/8" dia. steel ball—15 kgm. load) |                |              |                   |                   |                   |                   |                   |
|--------------------------------------|-------|---------------------------------------------------------------------------------|----------------|--------------|-------------------|-------------------|-------------------|-------------------|-------------------|
| Individual                           | Total | $R_w$ as Pressed                                                                | $R_w$ Sintered | $R_w$ Coined | $R_w$ @ 1,000° F. | $R_w$ @ 1,100° F. | $R_w$ @ 1,150° F. | $R_w$ @ 1,200° F. | $R_w$ @ 1,250° F. |
| Pure Aluminum                        |       | 88                                                                              | 89             | 93           | 66                | 50                | 23                |                   |                   |
| TiO <sub>2</sub>                     | 5     | 86                                                                              | 88             | 90           | 67                | 56                | 28                | off scale         |                   |
| TiO <sub>2</sub>                     | 10    | 87                                                                              | 90             | 90           | 70                | 55                | 36                | <10               |                   |
| TiO <sub>2</sub>                     | 25    | 87                                                                              | 92             | 92           | 73                | 73                | 54                | 56                | 22                |
| TiO <sub>2</sub>                     | 50    | 84                                                                              | 90             | 90           | 77                | 82                | 79                |                   | 72                |
| Fe <sub>2</sub> O <sub>3</sub>       | 5     | 87                                                                              | 84             | 89           | 67                | 60                | 46                | 41                |                   |
| V <sub>2</sub> O <sub>5</sub>        | 5     | 87                                                                              | 84             | 89           | 63                | 48                | 28                |                   |                   |
| V <sub>2</sub> O <sub>5</sub>        | 10    | 87                                                                              | 81             | 88           | 62                | 55                | 36                |                   |                   |
| V <sub>2</sub> O <sub>5</sub>        | 25    | 69                                                                              | 69             | 87           | 67                | 62                | 52                | 40                |                   |
| Cr <sub>2</sub> O <sub>3</sub>       | 5     | 88                                                                              | 87             | 88           | 69                | 50                | 35                |                   |                   |
| Cr <sub>2</sub> O <sub>3</sub>       | 10    | 85                                                                              | 85             | 89           | 67                | 48                | 42                |                   |                   |
| Cr <sub>2</sub> O <sub>3</sub>       | 25    | 87                                                                              | 86             | 88           | 70                | 59                | 68                | 42                |                   |
| ZrO <sub>2</sub>                     | 5     | 85                                                                              | 84             | 88           | 64                | 55                | 27                |                   |                   |
| ZrO <sub>2</sub>                     | 10    | 84                                                                              | 86             | 88           | 61                | 41                | 43                | off scale         |                   |
| ZrO <sub>2</sub>                     | 25    | 84                                                                              | 86             | 88           | 65                | 59                | 38                | 39                |                   |
| PrO                                  | 5     | 88                                                                              | 85             | 90           | 70                | 52                | 25                |                   |                   |
| PrO                                  | 10    | 88                                                                              | 85             | 87           | 66                | 52                | 25                |                   |                   |
| PrO                                  | 25    | 83                                                                              | 79             | 87           | 70                | 61                | 52                | 50                |                   |
| Mo <sub>2</sub> O <sub>5</sub>       | 5     | 85                                                                              | 83             | 89           | 65                | 62                | 57                | 21                |                   |
| MgO                                  | 5     | 85                                                                              | 86             | 89           |                   |                   |                   |                   |                   |
| MgO                                  | 10    | 85                                                                              | 86             | 90           |                   |                   |                   |                   |                   |
| MgO                                  | 25    | 85                                                                              | 85             | 89           |                   |                   |                   |                   |                   |
| BaS                                  | 5     | 84                                                                              | 86             | 87           |                   |                   |                   |                   |                   |
| BaS                                  | 10    | 84                                                                              | 85             | 88           |                   |                   |                   |                   |                   |
| MoS <sub>2</sub>                     | 5     | 81                                                                              | 85             | 89           |                   |                   |                   |                   |                   |
| SiC                                  | 5     | 84                                                                              | 87             | 90           |                   |                   |                   |                   |                   |
| SiC                                  | 10    | 88                                                                              | 86             | 90           |                   |                   |                   |                   |                   |
| SiC                                  | 25    | 83                                                                              | 86             | 90           |                   |                   |                   |                   |                   |
| Zr Boride                            | 5     | 84                                                                              | 86             | 90           | 64                | 46                | 30                |                   |                   |
| Zr Boride                            | 10    | 84                                                                              | 85             | 89           | 67                | 40                | 29                |                   |                   |
| Zr Boride                            | 25    | 86                                                                              | 86             | 89           | 67                | 47                | 31                |                   |                   |
| Fe                                   | 5     | 88                                                                              | 81             | 90           | 70                | 60                | 52                | 48                |                   |
| Fe                                   | 10    | 89                                                                              | 85             | 92           | 65                | 55                | 47                | 41                |                   |
| Ta                                   | 5     | 87                                                                              | 89             | 90           | 71                | 51                | 30                |                   |                   |
| Ta                                   | 10    | 82                                                                              | 86             | 90           | 70                | 50                | 30                |                   |                   |
| Ta                                   | 25    | 80                                                                              | 87             | 90           | 68                | 49                | 53                | off scale         |                   |
| Mo                                   | 5     | 87                                                                              |                |              |                   |                   |                   |                   |                   |
| Mo                                   | 10    | 85                                                                              |                |              |                   |                   |                   |                   |                   |
| Mo                                   | 25    | 85                                                                              |                |              |                   |                   |                   |                   |                   |
| MnO <sub>2</sub>                     | 10    | 88                                                                              | 88             | 90           |                   |                   |                   |                   |                   |
| MnO <sub>2</sub>                     | 25    | 87                                                                              |                |              |                   |                   |                   |                   |                   |
| 2.5% Al <sub>2</sub> O <sub>3</sub>  |       |                                                                                 |                |              |                   |                   |                   |                   |                   |
| 2.5% TiO <sub>2</sub>                | 5     | 81                                                                              | 86             | 89           | 72                | 60                | 36                | off scale         |                   |
| 5% Al <sub>2</sub> O <sub>3</sub>    |       |                                                                                 |                |              |                   |                   |                   |                   |                   |
| 5% TiO <sub>2</sub>                  | 10    | 87                                                                              | 88             | 89           | 64                | 50                | 26                | off scale         |                   |
| 12.5% Al <sub>2</sub> O <sub>3</sub> |       |                                                                                 |                |              |                   |                   |                   |                   |                   |
| 12.5% TiO <sub>2</sub>               | 25    | 89                                                                              | 89             | 90           | 74                | 56                | 44                |                   |                   |
| 25% Al <sub>2</sub> O <sub>3</sub>   |       |                                                                                 |                |              |                   |                   |                   |                   |                   |
| 25% TiO <sub>2</sub>                 | 50    | 86                                                                              | 88             | 89           | 86                | 80                | 79                | 74                | 76                |
| 5% MnO <sub>2</sub>                  |       |                                                                                 |                |              |                   |                   |                   |                   |                   |
| 5% V <sub>2</sub> O <sub>5</sub>     | 10    | 87                                                                              |                |              |                   |                   |                   |                   |                   |
| 5% MnO <sub>2</sub>                  |       |                                                                                 |                |              |                   |                   |                   |                   |                   |
| 5% Al <sub>2</sub> O <sub>3</sub>    |       |                                                                                 |                |              |                   |                   |                   |                   |                   |
| 1.7% MnO <sub>2</sub>                |       |                                                                                 |                |              |                   |                   |                   |                   |                   |
| 1.7% V <sub>2</sub> O <sub>5</sub>   | 5.1   | 87                                                                              | 88             | 89           |                   |                   |                   |                   |                   |
| 1.7% Al <sub>2</sub> O <sub>3</sub>  |       |                                                                                 |                |              |                   |                   |                   |                   |                   |
| 12.5% TiO <sub>2</sub>               |       |                                                                                 |                |              |                   |                   |                   |                   |                   |
| 12.5% V <sub>2</sub> O <sub>5</sub>  | 25    | 86                                                                              | 87             | 89           |                   |                   |                   |                   |                   |
| 6.5% V <sub>2</sub> O <sub>5</sub>   |       |                                                                                 |                |              |                   |                   |                   |                   |                   |
| 6.5% MgO                             |       |                                                                                 |                |              |                   |                   |                   |                   |                   |
| 6.5% Al <sub>2</sub> O <sub>3</sub>  |       |                                                                                 |                |              |                   |                   |                   |                   |                   |
| 6.5% TiO <sub>2</sub>                |       |                                                                                 |                |              |                   |                   |                   |                   |                   |
| CaTiO <sub>3</sub>                   | 5     |                                                                                 |                |              |                   |                   |                   |                   |                   |
| CaTiO <sub>3</sub>                   | 10    |                                                                                 |                |              |                   |                   |                   |                   |                   |
| CaTiO <sub>3</sub>                   | 25    |                                                                                 |                |              |                   |                   |                   |                   |                   |
| BaTiO <sub>3</sub>                   | 5     |                                                                                 |                |              |                   |                   |                   |                   |                   |
| BaTiO <sub>3</sub>                   | 10    |                                                                                 |                |              |                   |                   |                   |                   |                   |
| BaTiO <sub>3</sub>                   | 25    |                                                                                 |                |              |                   |                   |                   |                   |                   |
| 12.5% MnO <sub>2</sub>               |       |                                                                                 |                |              |                   |                   |                   |                   |                   |
| 12.5% V <sub>2</sub> O <sub>5</sub>  | 25    | 87                                                                              |                |              |                   |                   |                   |                   |                   |
| 2.5% CaTiO <sub>3</sub>              |       |                                                                                 |                |              |                   |                   |                   |                   |                   |
| 2.5% TiO <sub>2</sub>                | 5     |                                                                                 |                |              |                   |                   |                   |                   |                   |
| 5% CaTiO <sub>3</sub>                |       |                                                                                 |                |              |                   |                   |                   |                   |                   |
| 5% TiO <sub>2</sub>                  | 10    |                                                                                 |                |              |                   |                   |                   |                   |                   |
| 12.5% CaTiO <sub>3</sub>             |       |                                                                                 |                |              |                   |                   |                   |                   |                   |
| 12.5% TiO <sub>2</sub>               | 25    |                                                                                 |                |              |                   |                   |                   |                   |                   |
| 2.5% BaTiO <sub>3</sub>              | 5     |                                                                                 |                |              |                   |                   |                   |                   |                   |
| 5% BaTiO <sub>3</sub>                |       |                                                                                 |                |              |                   |                   |                   |                   |                   |
| 5% TiO <sub>2</sub>                  | 10    |                                                                                 |                |              |                   |                   |                   |                   |                   |
| 12.5% BaTiO <sub>3</sub>             |       |                                                                                 |                |              |                   |                   |                   |                   |                   |
| 12.5% TiO <sub>2</sub>               | 25    |                                                                                 |                |              |                   |                   |                   |                   |                   |

It is apparent from Table I that many different inorganic substances may be added to aluminum powder to increase hardness and strength at elevated temperatures of products made from the composite powder. Metal oxide additives and mixtures thereof have generally proven to be very effective in retaining hardness and strength in aluminum for most purposes. Those oxides found to

be highly effective are titanium dioxide, a titanium dioxide-aluminum oxide mixture, magnesium oxide, chromic oxide, praseodymium oxide, and molybdenum, sesquioxide.

The simple metal oxide additives found to be useful for the purpose of this invention are those inorganic oxides of metals other than aluminum which are stable and

not appreciably reactive with aluminum or oxygen at temperatures up to about 1200° F., and mixtures of one or more of such oxides with or without aluminum oxide.

The compounds of mixed oxides useful as additives to aluminum or aluminum alloy powder for the purpose of the invention may be defined as those inorganic compounds of mixed oxides which are stable and not appreciably reactive with aluminum or oxygen at temperatures up to about 1200° F., and mixtures of one or more of such mixed oxides. An example of one such compound is calcium titanate,  $\text{CaTiO}_3$ , which may be considered as a compound of calcium oxide and titanium dioxide,  $\text{CaO}\cdot\text{TiO}_2$ , for the purposes of the invention. Other examples are aluminates, titanate, silicates, and analogous compounds of vanadium, chromium and nickel.

The metal powders useful as additives to aluminum powder compositions in accordance with the invention are metals known in the art as strengthening metals for aluminum alloys. Examples of such metals are Fe, Mo, V, Ti, Ta, Cb, Cr, Mn, Ni, W, B, and rare earth elements.

It is understood that mixtures comprising one or more of the before mentioned metals, simple metal oxides, or mixed metal oxides are useful as additives, as well as metal sulfides, carbides, borides, and inorganic oxygen bearing compounds which do not decompose or react appreciably with aluminum or oxygen at temperatures up to about 1200° F.

In order to obtain the improvement in properties of aluminum based powder products described herein, it appears desirable that the fine aluminum particles be uniformly surrounded by non-reactive heat-stable inorganic barriers to the diffusion of aluminum atoms. Additives which decompose upon heating or react appreciably with aluminum or oxygen at temperatures up to about 1200° F. reduce hot hardness and strength, and in some instances destroy the completed product as a result of the reaction.

The most satisfactory aluminum powder for use in powder compositions of the invention is very finely divided (1% retained on 325 mesh screen) low lubricant flake aluminum powder. It is also highly desirable that additives thereto be in a finely divided state. An additive particle size of 5-50 microns was found to be suitable, but no particular correlation was found between particle

size and hardness. However, all satisfactory additives were quite fine powders, as shown by Table II.

Table II gives the Rockwell hardness value (Rw) at 1120° F. and compressive strength (CS) in pounds per square inch at 70° F. for aluminum base powder products composed of low lubricant flake aluminum powder (1% retained on 325 mesh screen) and additives in percentages by weight having various particle sizes in microns ( $\mu$ ). The Rockwell hardness values (Rw) for Table II, as well as Table I, were obtained by following the testing procedure to be described in the example. The compressive strength (CS) was obtained by inserting experimental data in the formula  $CS = P/A$  and making computations therefrom, where P is the maximum lead before failure in pounds and A is the cross-sectional area of the aluminum base powder product in square inches.

The following specific example of the invention for preparing a metallurgical powder composition and manufacture of a form therefrom is given for purposes of illustration only:

#### Example

#### PREPARATION OF POWDER

A dry powder composition was prepared from 50% (by weight) low lubricant flake aluminum powder (1% retained on 325 mesh screen) and 50% finely divided titanium dioxide (average particle size  $50\mu$ ).

In order to press the powder composition it was found desirable to ball mill (mill capacity 1000 cc., containing 165 $\frac{1}{2}$  and 140 $\frac{1}{2}$  steel balls, speed of rotation 96 R. P. M.) a 40 gm. powder charge with sufficient wetting agent (xylene) to form a soft paste (25-60 cc.).

The milled charge was removed from the ball mill, separated from the steel balls, then placed in an aluminum boat and pre-sintered for one hour at 800° F. under inert (argon) atmosphere. The charge was cooled to room temperature before exposing to air.

#### MANUFACTURE AND PROCESSING OF COMPACTS

The powder composition as above prepared was found to be readily pressed. A compact was made using a double action die and a pressure of 40 tons p. s. i. Pres-

TABLE II. — PARTICLE SIZE OF ADDITIONS, HARDNESS @ 1120° F. AND COMPRESSIVE STRENGTH OF ALUMINUM BASE POWDER PRODUCTS

| Addition                               | Size Range ( $\mu$ ) | Avg. Size ( $\mu$ ) | Hardness @ 1,120° F.; Compressive Strength @ 70° F. |                                     |              |                                     |              |                                     |              |                                     |
|----------------------------------------|----------------------|---------------------|-----------------------------------------------------|-------------------------------------|--------------|-------------------------------------|--------------|-------------------------------------|--------------|-------------------------------------|
|                                        |                      |                     | 5% Addition                                         |                                     | 10% Addition |                                     | 25% Addition |                                     | 50% Addition |                                     |
|                                        |                      |                     | Rw                                                  | C. S.,<br>p. s. i. $\times 10^{-3}$ | Rw           | C. S.,<br>p. s. i. $\times 10^{-3}$ | Rw           | C. S.,<br>p. s. i. $\times 10^{-3}$ | Rw           | C. S.,<br>p. s. i. $\times 10^{-3}$ |
| $\text{TiO}_2$                         | 25-100               | 50                  | 32                                                  | 56.6                                | 36           | 56.0                                | 58           | 52.0                                | 75           | 30.9                                |
| B                                      | 5-25                 | 12.5                | 33                                                  | 51.6                                | 40           | 51.0                                | 52           | 47.7                                | -----        | -----                               |
| ZrB                                    | 5-25                 | 12.5                | 45                                                  | 60.0                                | 42           | 47.8                                | 45           | 50.6                                | -----        | -----                               |
| $\text{Al}_2\text{O}_3 + \text{TiO}_2$ | -----                | 48                  | 48.5                                                | 47                                  | 51.0         | 53                                  | 49.0         | 77                                  | 35.3         | -----                               |
| $\text{Fe}_2\text{O}_4$                | 2.5-12.5             | 5                   | 58                                                  | 49.8                                | -----        | -----                               | 27           | 41.6                                | -----        | -----                               |
| $\text{V}_2\text{O}_5$                 | 7.5-50               | 25                  | 37                                                  | 62.6                                | 29           | 58.3                                | 54           | 43.6                                | -----        | -----                               |
| Fe                                     | 2.5-12.5             | 7.5                 | 46                                                  | 52.8                                | 57           | 49.2                                | -----        | -----                               | -----        | -----                               |
| Ta                                     | 25-100               | 50                  | 30                                                  | 57.0                                | 35           | 53.6                                | -----        | -----                               | -----        | -----                               |
| AlC                                    | 2.5-12.5             | 5                   | -----                                               | -----                               | -----        | -----                               | 27           | 41.6                                | -----        | -----                               |
| $\text{CeO}_2$                         | 2.5-25               | 12.5                | 25                                                  | 53.4                                | 36           | 51.4                                | 25           | 52.8                                | -----        | -----                               |
| $\text{LaO}$                           | 2.5-50               | 12.5                | 34                                                  | 51.9                                | 45           | 49.2                                | 39           | 32.5                                | -----        | -----                               |
| $\text{Cr}_2\text{O}_3$                | 2.5-25               | 1.25                | 49                                                  | 51.5                                | 50           | 53.2                                | 59           | 54.9                                | -----        | -----                               |
| $\text{ZrO}_2$                         | 25-12.5              | 2.5                 | 42                                                  | 53.4                                | 44           | 53.8                                | 53           | 52.1                                | -----        | -----                               |
| $\text{PrO}$                           | 2.5-25               | 12.5                | 25                                                  | 52.4                                | 25           | 50.9                                | 60           | 45.4                                | -----        | -----                               |
| $\text{Mo}_2\text{O}_5$                | 2.5-25               | 12.5                | 36                                                  | 54.3                                | -----        | -----                               | -----        | -----                               | -----        | -----                               |
| Sb                                     | 2.5-35               | 12.5                | -----                                               | -----                               | 36           | 56.4                                | 33           | 58.5                                | -----        | -----                               |
| Mo                                     | 2.5-12.5             | 5                   | 46                                                  | 50.2                                | 46           | 54.6                                | 42           | 56.5                                | -----        | -----                               |
| $\text{BaS}_2$                         | 2.5-35               | 12.5                | 42                                                  | 53.3                                | 48           | 51.5                                | -----        | -----                               | -----        | -----                               |
| $\text{MoS}_2$                         | 2.5-12.5             | 50                  | 51                                                  | 51.8                                | -----        | -----                               | -----        | -----                               | -----        | -----                               |
| $\text{MgO}$                           | 2.5-50               | 7.5                 | 42                                                  | 50.4                                | 45           | 49.2                                | 70           | 39.1                                | -----        | -----                               |
| SiC                                    | 5-50                 | 25                  | 31                                                  | 54.0                                | 33           | 53.0                                | 31           | 46.6                                | -----        | -----                               |

sures greater than this caused welding of the aluminum to the walls of the die and eventually resulted in fracturing of the die, as well as cracking of the specimen upon ejection from the die.

A sintering step was carried out at 1000-1050° F. for one hour under inert (argon) atmosphere, followed by air cooling to room temperature.

It was found that compacts harder at room temperature were also harder at elevated temperatures. Accordingly, all compacts were repressed after sintering by a process known as coining, and in the same die used for making the compacts.

It was noted in most instances that due to cold welding, the pressed compacts were about as hard as after complete processing. Where cold welding is achieved during the pressing step, it appears that the sintering step may be omitted in some instances.

#### TESTING OF COMPACTS

Hot hardness testing of the products as above prepared was chosen because of the well known correlation between hot hardness, creep, and creep-rupture strength. Compacts prepared in accordance with the invention, as previously described, were hot tested using a Rockwell Superficial Hardness tester with a 15 kg. load and  $\frac{1}{8}$ " steel ball indenter (Rockwell w scale). The anvils were cylindrical stainless steel blocks 3" in height and  $2\frac{1}{2}$ " in diameter with cylindrical cavities in the top. A larger anvil was used to support the stainless steel block with a  $\frac{1}{4}$ " sheet of transite interposed between the larger anvil and stainless steel block.

The stainless steel blocks were heated to testing temperature and a compact specimen placed in the cavity. The assembly was furnace-heated to testing temperature and the temperature maintained for a period of one hour. The assembly was then removed from the furnace to the Rockwell Superficial Hardness tester and readings (Rockwell w scale) taken as rapidly as possible.

It is to be understood that the invention is not limited to aluminum or aluminum alloy powder as the basic metallic component of the described metallurgical powder compositions, or to the preparation of such powder compositions by the described addition of powdered additives. Aluminum powder or other metallic powder, or aluminum flake or other metallic flake, and mixtures thereof may be either admixed or coated with metal additive or other inorganic additive described hereinto produce the metallurgical powder compositions of the invention. Alternatively, the basic metallic component of powder compositions may be coated with inorganic additive by any suitable well known method of coating metals, such as by means of vapor or vacuum deposition, or electroplating. The powder compositions, whether the basic metallic component is admixed or coated with inorganic additive, may be processed into a body of desired size and shape by the described method or by other suitable well known methods not specifically described herein. For example, depending upon the characteristics of the particular powder composition, cold pressing or hot pressing alone may be sufficient, or cold pressing in combination with sintering and/or hot pressing, or a combination of the foregoing steps, or by hot extrusion.

Obviously many modifications and variations of the present invention are possible in the light of the above teachings. It is, therefore, to be understood that within the scope of the appended claims the invention may be practiced otherwise than as specifically described.

What is claimed as new and desired to be secured by Letters Patent of the United States is:

1. A metallurgical composition for use in the production of structural material capable of unusual strength and hardness up to about 1200° F. comprising an intimate finely divided mixture consisting of 75 to 95 parts by weight of a metallic base selected from the group consisting of aluminum and alloys of aluminum, and 25 to 5

parts by weight of an additive selected from the group consisting of the inorganic oxygen bearing compounds of a metal selected from the group consisting of magnesium, titanium, vanadium, chromium, zirconium, lanthanum, cerium and praseodymium, which compounds do not contain any non-metal other than oxygen mixtures of said compounds, mixtures of said compounds with aluminum alloy strengthening metals selected from the group consisting of iron, molybdenum, vanadium, titanium, tantalum, columbium, chromium, manganese, nickel, tungsten, boron and the rare earth elements, mixtures of said compounds with aluminum oxide, and mixtures of said compounds with said strengthening metals and aluminum oxide, said inorganic oxygen bearing compound comprising at least 5 parts by weight of said composition.

2. The metallurgical composition of claim 1 wherein the inorganic oxygen bearing compound is a compound of titanium.

3. The metallurgical composition of claim 1 wherein the additive contains aluminum oxide.

4. A structural material formed by mechanical working under pressure from a finely divided mixture of 75 to 95 parts by weight of a metallic base selected from the group consisting of aluminum and alloys of aluminum and 25 to 5 parts by weight of an additive selected from the group consisting of the inorganic oxygen bearing compounds of a metal selected from the group consisting of magnesium, titanium, vanadium, chromium, zirconium, lanthanum, cerium and praseodymium, which compounds

do not contain any non-metal other than oxygen, mixtures of said compounds, mixtures of said compounds with aluminum alloy strengthening metals selected from the group consisting of iron, molybdenum, vanadium, titanium, tantalum, columbium, chromium, manganese, nickel, tungsten, boron and the rare earth elements, and mixtures of said compounds with aluminum oxide, said inorganic oxygen bearing compound comprising at least 5 parts by weight of said composition, said finely divided mixture having been heated under non-oxidizing conditions to a temperature between about 800° F. and about the melting point of aluminum.

5. A structural material formed by mechanical working under pressure from a finely divided mixture of 75 to 95 parts by weight of a metallic base selected from the group consisting of aluminum and alloys of aluminum and 25 to 5 parts by weight of an additive selected from the group consisting of the inorganic oxygen bearing compounds of a metal selected from the group consisting of magnesium, titanium, vanadium, chromium, zirconium, lanthanum, cerium and praseodymium, which compounds

do not contain any non-metal other than oxygen, mixtures of said compounds, mixtures of said compounds with aluminum alloy strengthening metals selected from the group consisting of iron, molybdenum, vanadium, titanium, tantalum, columbium, chromium, manganese, nickel, tungsten, boron and the rare earth elements, and mixtures of said compounds with aluminum oxide, said inorganic oxygen bearing compounds comprising at least 5 parts by weight of said composition, said finely divided mixture having been heated under non-oxidizing conditions to a temperature between about 800° F. and about the melting point of aluminum.

6. The structural material of claim 5 wherein the inorganic oxygen bearing compound is a compound of titanium.

7. The structural material of claim 5 wherein the additive contains aluminum oxide.

8. The method of producing a structural material capable of unusual strength and hardness up to about 1200° F. by heating under non-oxidizing conditions to a temperature from about 800° F. to about the melting point of aluminum a finely divided mixture of 75 to 95 parts by weight of a metallic base selected from the group consisting of aluminum and alloys of aluminum and 25 to 5 parts by weight of an additive selected from the group

consisting of the inorganic oxygen bearing compounds of a metal selected from the group consisting of magnesium, titanium, vanadium, chromium, zirconium, lanthanum, cerium and praseodymium, which compounds do not contain any non-metals other than oxygen, mixtures of said compounds, mixtures of said compounds with aluminum alloy strengthening metals selected from the group consisting of iron, molybdenum, vanadium, titanium, tantalum, columbium, chromium, manganese, nickel, tungsten, boron and the rare earth elements, mixtures of said compounds with said strengthening metals and mixtures of said compounds with aluminum oxide, said inorganic oxygen bearing compound comprising at least 5 parts by weight of said composition, and mechanically working said mixture under pressure to form said material.

## References Cited in the file of this patent

## UNITED STATES PATENTS

|           |          |                |
|-----------|----------|----------------|
| 2,568,157 | Lepp     | Sept. 18, 1951 |
| 2,613,153 | Stafford | Oct. 7, 1952   |

## FOREIGN PATENTS

|         |               |                |
|---------|---------------|----------------|
| 517,773 | Great Britain | Feb. 8, 1940   |
| 910,811 | France        | Feb. 18, 1946  |
| 625,364 | Great Britain | June 27, 1949  |
| 490,455 | Canada        | Feb. 10, 1953  |
| 176,025 | Austria       | Sept. 10, 1953 |
| 897,715 | Germany       | Nov. 23, 1953  |

## OTHER REFERENCES

"Metal Powder Report," vol. 4, No. 8, April 1950, page 126.

UNITED STATES PATENT OFFICE  
CERTIFICATE OF CORRECTION

July 1, 1958

Patent No. 2,840,891

John S. Nachtman

It is hereby certified that error appears in the printed specification of the above numbered patent requiring correction and that the said Letters Patent should read as corrected below.

Column 8, line 6, for "oxygen mixtures" read -- oxygen, mixtures --.

Signed and sealed this 9th day of December 1958.

(SEAL)

Attest:

KARL H. AXLINE

Attesting Officer

ROBERT C. WATSON  
Commissioner of Patents